

# UNITED STATES PATENT OFFICE.

ALBERT L. MARSH, OF DETROIT, MICHIGAN, ASSIGNOR TO HOSKINS MANUFACTURING COMPANY, OF DETROIT, MICHIGAN, A CORPORATION OF MICHIGAN.

## LABORATORY UTENSIL-HOLDER.

1,012,391.

Specification of Letters Patent. Patented Dec. 19, 1911.

No Drawing.

Application filed November 11, 1910. Serial No. 591,911.

*To all whom it may concern:*

Be it known that I, ALBERT L. MARSH, a citizen of the United States, residing at Detroit, in the county of Wayne and State of Michigan, have invented a new and useful Improvement in Laboratory Utensil-Holders, of which the following is a specification.

The object of my invention is to provide holders, such as triangles, crucible-tongs tips, wire-gauze, and the like, employed in metallurgical laboratory work for supporting and handling the work, which shall enduringly withstand the destructive tendency 10 of the high temperature to which they are subjected in use to destroy them and be particularly suitable for quantitative analytical work. When such holders are made of any base metal, the heat to which they are 15 subjected in use rapidly destroys them by oxidation, and the metal, in being brought into contact with the heated platinum or porcelain of which the crucibles and other ware are made, discolors the surfaces, adding 20 to the weight of the ware and thus rendering such holders unfit for quantitative analytical work. To avoid, more particularly, the last-named objection, such holders are sometimes made of platinum 25 because it remains unaffected by the heat, but its cost renders it practically prohibitive for the purpose; and to enable a base metal to be used for avoiding that objection, sheathing the holder with fire-clay, 30 fused silica, or the like, has been resorted to, but the metal soon "burns out," so that the holder is lacking in desirable durability.

My invention provides a holder, in the class referred to, which is devoid of these 35 objections, and it consists in forming such holders of an alloy containing nickel or cobalt with chromium, and preferably also aluminum. I find that a holder composed of such an alloy effectually resists destruction by heat, and remains otherwise unaffected injuriously thereby during prolonged use, because of the very high melt-

ing point of the nickel or cobalt and the property of the chromium of reducing to the minimum the tendency of the nickel or cobalt to oxidize. The value, for my purpose, of aluminum as a part of the alloy is its effect under the influence of intense heat to produce an oxid which, combining with the oxids produced by the same influence from the other metals in the alloy, forms a continuous, very thin, dense and adherent non-scaling sheath or surface-coating, which protects the holder by insulating the body or interior of the structure against further oxidizing influence thereon. Moreover, the holder does not discolor. The alloy is best suited for my improved article of holder, as imparting to it in the highest degree the desirable property herein described, when composed of about eighty per cent. nickel or cobalt, about eighteen per cent. chromium and about two per cent. aluminum.

What I claim as new and desire to secure by Letters Patent is—

1. A holder having the properties set forth, for receptacles employed in metallurgical laboratory work of the character described, formed of an alloy of chromium with a metal having the properties of nickel and cobalt.

2. A holder having the properties set forth, for receptacles employed in metallurgical laboratory work of the character described, formed of an alloy of nickel, chromium and aluminum.

3. A holder having the properties set forth, for receptacles employed in metallurgical laboratory work of the character described, formed of an alloy composed of nickel in the proportion of about eighty per cent., chromium in the proportion of about eighteen per cent., and aluminum in the proportion of about two per cent.

ALBERT L. MARSH.

In presence of—

A. G. MELCHER,  
Wm. A. TALMAN.